# EUROPEAN PATENT APPLICATION

(11) **EP 4 678 773 A1**
(43) Date of publication of application: **14.01.2026**
(21) Application number: 24767114.2
(22) Date of filing: 04.03.2024
(51) Int. Cl.: C22C 30/00, C22C 30/02, C22F 1/00, C22F 1/10

(54) **AUSTENITE-BASED HEAT-RESISTANT ALLOY MEMBER**

(30) Priority: 07.03.2023 JP 2023034369
(71) Applicant: NIPPON STEEL CORPORATION, Tokyo 100-8071 (JP)
(72) Inventor: HAMAGUCHI, Tomoaki, Tokyo 100-8071 (JP); OTAKI, Nao, Tokyo 100-8071 (JP); TANAKA, Katsuki, Tokyo 100-8071 (JP)
(74) Representative: Zimmermann & Partner Patentanwälte mbB
(86) International application number: PCT/JP2024/008081
(87) International publication number: WO 2024/185746

(57) **Abstract**

An austenitic heat resistant alloy member having a chemical composition including, in mass%: C: 0.010 to 0.150%, Si: 2.00% or less, Mn: 2.00% or less, P: 0.0400% or less, S: 0.0100% or less, Cr: 20.00 to 28.00%, Ni: 35.00 to 50.00%, W: 4.00 to 10.00%, Ti: 0.01 to 1.20%, Nb: 0.01 to 1.00%, N: 0.0200% or less, Al: 0.010 to 0.300%, B: 0.0005 to 0.0400%, O: 0.0100% or less, and the balance: Fe and impurities, and satisfies 97.50 ≤ (Cr+W+Fe+Ni) - (Cr_{ER}+W_{ER}+Fe_{ER}+Ni_{ER}) and -2.2×10⁻⁵×t³+2.1≤D.

## Description

### TECHNICAL FIELD

The present invention relates to an austenitic heat resistant alloy member.

### BACKGROUND ART

Recently, from the viewpoint of reducing environmental burden, power generation boilers and the like are increasingly operated under conditions of higher temperatures and pressures on a global scale. Austenitic heat resistant alloy members used as materials for superheater tubes and reheater tubes are required to have more excellent creep rupture strength.

Given such a technical background, there have been proposed techniques related to various austenitic heat resistant alloys. For example, Patent Document 1 discloses an austenitic heat resistant alloy member that has both excellent hot workability and creep rupture strength, which are achieved by strictly controlling the content of S relative to the contents of Ca, Mg, and REM.

In addition, Patent Document 2 discloses an austenitic heat resistant alloy, and a production method of the same, in which a 0.2% yield stress and a tensile strength sufficient for large structural members at normal temperature and a creep rupture strength at high temperature become evident by carrying out a heat treatment under suitable conditions to reduce variation in mechanical properties depending on locations.

Furthermore, Patent Document 3 discloses an austenitic heat resistant alloy member that has a thickness exceeding 30 mm and that has an improved creep strength and crack resistance during welding when being subjected to multi-layer welding, which are achieved by controlling an average grain diameter at a thickness-center portion of a member depending on the contents of B, Ti, and W.

Still further, Patent Document 4 discloses an austenitic stainless steel that has an improved high-temperature strength and fatigue resistance, which are achieved by increasing the content of W, which is effective for increasing the strength, to generate a microstructure that has coarse austenite grains and less variation.

### LIST OF PRIOR ART DOCUMENTS

### PATENT DOCUMENT

Patent Document 1: JP2017-206717A
Patent Document 2: WO 2018/146783
Patent Document 3: JP2014-141713A
Patent Document 4: JP2004-3000A

### SUMMARY OF INVENTION

### TECHNICAL PROBLEM

However, in the case of a steel with emphasis on the improvement of the creep rupture strength, it has been revealed that the creep rupture ductility for long-term at high temperature may be slightly lower in some cases. Accordingly, in the prior arts, further improvement is still necessary from the viewpoint of achieving both a high creep rupture strength and a high creep rupture ductility.

An objective of the present invention is to solve the above-described problems and provide an austenitic heat resistant alloy member that is excellent in both the creep rupture strength and the creep rupture ductility.

### SOLUTION TO PROBLEM

To solve the above-described problems, the inventors have conducted detailed studies on the creep rupture strength and the creep rupture ductility, and as a result, obtained the following findings.
(a) It has been found that in an alloy member that has an excellent creep rupture strength, precipitates that contain Cr, W, Fe, and/or Ni have finely precipitated in a usage environment. Then, for causing these elements to finely precipitate in a usage environment, it is important to perform a solution heat treatment in advance such that Cr, W, Fe, and Ni are sufficiently dissolved.
(b) On the other hand, an excessive solution heat treatment leads to coarsening of austenite grains, so that the creep rupture ductility degrades. Accordingly, it is necessary to appropriately adjust the solution heat treatment conditions.
(c) However, the solution heat treatment conditions for sufficiently dissolving Cr, W, Fe, and Ni along the thickness direction of the member depend on the thickness of the member. The inventors have then conducted detailed studies on the creep rupture ductility for members that have various thicknesses. As a result, the inventors have found that there is a certain relationship between the thickness of a member and the grain size number that leads to a better creep rupture ductility. Accordingly, to achieve both an excellent creep rupture strength and creep rupture ductility, it is necessary to strictly control the solution heat treatment conditions in consideration of the thickness of the member.

The gist of the present invention, which has been completed based on the above-described findings, is an austenitic heat resistant alloy member described below.
(1) An austenitic heat resistant alloy member having a chemical composition including, in mass%:
   C: 0.010 to 0.150%,
   Si: 2.00% or less,
   Mn: 2.00% or less,
   P: 0.0400% or less,
   S: 0.0100% or less,
   Cr: 20.00 to 28.00%,
   Ni: 35.00 to 50.00%,
   W: 4.00 to 10.00%,
   Ti: 0.01 to 1.20%,
   Nb: 0.01 to 1.00%,
   N: 0.0200% or less,
   Al: 0.010 to 0.300%,
   B: 0.0005 to 0.0400%,
   O: 0.0100% or less, and
   the balance: Fe and impurities, and
   satisfies following Formulas (i) and (ii): $97.50 \leq \left(Cr+W+Fe+Ni\right) - \left({Cr}_{ER}+{W}_{ER}+{Fe}_{ER}+{Ni}_{ER}\right)$ $- 2.2 \times {10}^{- 5} \times {t}^{3} + 2.1 \leq D$
   where each symbol in the formulas is defined as below, and each element symbol in the formulas represents a content of each element (mass%) contained in the alloy member,
   Cr_{ER}: a content of Cr (mass%) in precipitates obtained by extracted residue analysis
   W_{ER}: a content of W (mass%) in precipitates obtained by extracted residue analysis
   Fe_{ER}: a content of Fe (mass%) in precipitates obtained by extracted residue analysis
   Ni_{ER}: a content of Ni (mass%) in precipitates obtained by extracted residue analysis
   t: a thickness of the alloy member (mm)
   D: an average grain size at a thickness-center portion of the alloy member.
(2) The austenitic heat resistant alloy member according to the above (1), wherein in lieu of a part of the Fe, the chemical composition contains one or more elements, in mass%, selected from:
   Ca: 0.0100% or less,
   Mg: 0.0500% or less,
   REM: 0.1000% or less,
   Co: 1.000% or less,
   Cu: 1.00% or less,
   Mo: 1.000% or less, and
   V: 0.500% or less.

### ADVANTAGEOUS EFFECTS OF INVENTION

The austenitic heat resistant alloy member of the present invention has both an excellent creep rupture strength and creep rupture ductility.

### DESCRIPTION OF EMBODIMENTS

The requirements for the present invention will now be described in detail.

### 1. Chemical Composition

The reason for limitation for each element is as described below. Note that in the description below, "%" for the content refers to "mass%".

### C: 0.010 to 0.150%

C (carbon) stabilizes the austenite and forms fine carbide in a grain boundary, leading to the improvement of the creep rupture strength at high temperature. To sufficiently obtain the effect, the content of C needs to be 0.010% or more. However, when C is excessively contained, the carbide will be coarsened and precipitate in large amounts, leading to the degradation of ductility of the grain boundary and also the degradation of toughness and the creep rupture strength. Accordingly, the content of C is 0.010 to 0.150%. The content of C is preferably 0.030% or more, and more preferably 0.050% or more. Furthermore, the content of C is preferably 0.120% or less, and more preferably 0.100% or less.

### Si: 2.00% or less

Si (silicon) has a deoxidation function and is an element that is effective for improving corrosion resistance and oxidation resistance at high temperature. However, when Si is excessively contained, the stability of the austenite degrades, leading to the degradation of toughness and the creep rupture strength. Accordingly, the content of Si is 2.00% or less. The content of Si is preferably 1.50% or less, and more preferably 1.00% or less.

It is not particularly necessary to provide a lower limit for the content of Si. However, excessive reduction of the content of Si leads to an insufficient deoxidation effect, and the level of cleanliness of alloy increases, leading to the degradation of cleanliness. Furthermore, it is difficult to produce the effect of improving corrosion resistance and oxidation resistance at high temperature, and production costs will significantly increase. Accordingly, the content of Si is preferably 0.02% or more, and more preferably 0.05% or more.

### Mn: 2.00% or less

As in Si, Mn (manganese) has not only a deoxidation function, but is also an element that contributes to stabilizing the austenite. However, an excessive content of Mn leads to embrittlement, and also the degradation of toughness and the creep rupture ductility. Accordingly, the content of Mn is 2.00% or less. The content of Mn is preferably 1.80% or less, and more preferably 1.50% or less.

It is not particularly necessary to provide a lower limit also for the content of Mn. However, excessive reduction of the content of Mn leads to an insufficient deoxidation effect, leading to the degradation of cleanliness of alloy. In addition, not only does hot workability degrade, but it is also difficult to produce the effect of stabilizing the austenite, and production costs will significantly increase. Accordingly, the content of Mn is preferably 0.005% or more, and more preferably 0.010% or more.

### P: 0.0400% or less

P (phosphorus) is contained as impurities in the alloy, and when contained in large amounts, leads to a significant degradation of hot workability and weldability, and also the degradation of the creep rupture ductility after being used for a long time. Accordingly, the content of P is 0.0400% or less. The content of P is preferably 0.0300% or less, and more preferably 0.0250% or less.

While it is preferable that the content of P is lowered as much as possible, excessive reduction leads to an increase in production costs. Accordingly, the content of P is preferably 0.0005% or more, and more preferably 0.0008% or more.

### S: 0.0100% or less

S (sulfur) produces an effect of improving creep rupture characteristics by being present in grains. However, when a large amount of S is contained, hot workability and weldability significantly degrade, and further the creep rupture ductility after being used for a long time degrades. Accordingly, the content of S is 0.0100% or less. The content of S is preferably 0.0095% or less, and more preferably 0.0090% or less.

When it is desirable to obtain an effect of improving the creep rupture characteristics by S, the content of S is preferably 0.0015% or more, more preferably 0.0018% or more, and further preferably 0.0020% or more.

### Cr: 20.00 to 28.00%

Cr (chromium) is dissolved in a matrix and is an element that significantly contributes to the improvement of the creep rupture strength at high temperature. Furthermore, Cr is an essential element for securing oxidation resistance and corrosion resistance at high temperature. To obtain the above-described effects, the content of Cr needs to be 20.00% or more. However, when the content of Cr exceeds 28.00%, the stability of the austenite at high temperature degrades, leading to the degradation of the creep rupture strength. Accordingly, the content of Cr is 20.00 to 28.00%. The content of Cr is preferably 21.00% or more, and more preferably 22.00% or more. Furthermore, the content of Cr is preferably 27.00% or less, and more preferably 26.00% or less.

### Ni: 35.00 to 50.00%

Ni (nickel) is dissolved in a matrix and is an element that significantly contributes to the improvement of the creep rupture strength at high temperature. Furthermore, Ni is an element that is effective for obtaining the austenite and is an essential element for securing the stability of the microstructure when being used for a long time. To sufficiently obtain the effect of Ni as described above to the extent of the above-described content of Cr, the content of Ni needs to be 35.00% or more. However, Ni is an expensive element, and when contained in large amounts, leads to an increase in costs. Accordingly, the content of Ni is 35.00 to 50.00%. The content of Ni is preferably 37.00% or more, and more preferably 39.00% or more. Furthermore, the content of Ni is preferably 48.00% or less, and more preferably 46.00% or less.

### W: 4.00 to 10.00%

W (tungsten) is dissolved in a matrix and is an element that significantly contributes to the improvement of the creep rupture strength at high temperature. To sufficiently produce the effect, the content of W needs to be 4.00% or more. However, excessively contained W leads only to the saturation of the effect, and what is worse, the creep rupture strength degrades. Furthermore, since W is an expensive element, costs will increase when excessively contained. Accordingly, the content of W is 4.00 to 10.00%. The content of W is preferably 5.00% or more, and more preferably 6.00% or more. Furthermore, the content of W is preferably 9.00% or less, and more preferably 8.00% or less.

### Ti: 0.01 to 1.20%

Ti (titanium) precipitates in grains as fine carbo-nitride and contributes to the improvement of the creep rupture strength at high temperature. To obtain the effects, the content of Ti needs to be 0.01% or more. However, an excessive content of Ti leads to the precipitation of a large amount of carbo-nitride and the degradation of the creep rupture ductility and toughness. Accordingly, the content of Ti is 0.01 to 1.20%. The content of Ti is preferably 0.03% or more, and more preferably 0.05% or more. Furthermore, the content of Ti is preferably 1.00% or less, and more preferably 0.80% or less.

### Nb: 0.01 to 1.00%

Nb (niobium) is combined with C, or C and N, precipitates in grains as fine carbide or carbo-nitride, and contributes to the improvement of the creep rupture strength at high temperature. To obtain the effects, the content of Nb needs to be 0.01% or more. However, an excessive content of Nb leads to the precipitation of a large amount of carbide carbo-nitride, and the degradation of the creep rupture ductility and toughness. Accordingly, the content of Nb is 0.01 to 1.00%. The content of Nb is preferably 0.05% or more, and more preferably 0.10% or more. Furthermore, the content of Nb is preferably 0.80% or less, and more preferably 0.60% or less.

### N: 0.0200% or less

N (nitrogen) is an element that is effective for stabilizing the austenite, whereas when excessively contained, a large amount of fine nitride precipitates in grains during the use at high temperature, leading to the degradation of the creep rupture ductility and toughness. Accordingly, the content of N is 0.0200% or less. The content of N is preferably 0.0180% or less, and more preferably 0.0150% or less.

It is not particularly necessary to provide a lower limit for the content of N. However, excessive reduction of the content of N leads to not only difficulty in obtaining an effect of stabilizing the austenite, but also a significant increase in production costs. Accordingly, the content of N is preferably 0.0005% or more, and more preferably 0.0008% or more.

### Al: 0.010 to 0.300%

Al (aluminum) is an element that has a deoxidation function, and therefore, the content of Al needs to be 0.010% or more. However, an excessive content of Al leads to a significant degradation of cleanliness of alloy, and the degradation of hot workability and ductility. Accordingly, the content of Al is 0.010 to 0.300%. The content of Al is preferably 0.030% or more, and more preferably 0.050% or more. Furthermore, the content of Al is preferably 0.250% or less, and more preferably 0.200% or less.

### B: 0.0005 to 0.0400%

B (boron) is an element that is necessary to improve the creep rupture strength by segregating in a grain boundary during the use at high temperature to strengthen the grain boundary and finely dispersing grain boundary carbide. To obtain the effects, the content of B needs to be 0.0005% or more. However, an excessive content of B leads to the degradation of weldability and the degradation of hot workability. Accordingly, the content of B is 0.0005 to 0.0400%. The content of B is preferably 0.0010% or more, and more preferably 0.0020% or more. Furthermore, the content of B is preferably 0.0300% or less, and more preferably 0.0200% or less.

### O: 0.0100% or less

O (oxygen) is contained in alloy as impurities, and an excessive content of O leads to the degradation of hot workability, and further the degradation of toughness and ductility. Accordingly, the content of O is 0.0100% or less. The content of O is preferably 0.0080% or less, and more preferably 0.0050% or less.

It is not particularly necessary to provide a lower limit for the content of O, whereas excessive reduction leads to an increase in production costs. Accordingly, the content of O is preferably 0.0005% or more, and more preferably 0.0008% or more.

In the chemical composition of the austenitic heat resistant alloy of the present invention, the balance is Fe and impurities. Here, "impurities" refer to components that are introduced due to various factors in raw materials such as ore and scrap and production processes when the alloy is industrially produced and that are acceptable to the extent that they do not adversely affect the present invention.

The austenitic heat resistant alloy of the present invention may further contain one or more elements selected from Ca, Mg, REM, Co, Cu, Mo, and V to the extent indicated below. Note that since these elements are not essential for the member, the lower limit value of the content is 0%. The reason for limitation for each element will be described.

### Ca: 0.0100% or less

Ca (calcium) forms a compound with S to reduce the amount of S in a matrix, producing an effect of improving hot workability, and therefore, Ca may be contained as necessary. However, an excessive content of Ca leads to a reduction in the amount of S in alloy that contributes to the improvement of the creep rupture strength, which is the advantageous effect of the present invention, and due to being combined with O, leads to a significant degradation of cleanliness, and what is worse, the degradation of hot workability. Accordingly, the content of Ca is 0.0100% or less. The content of Ca is preferably 0.0080% or less. When it is desirable to obtain the above-described effects, the content of Ca is preferably 0.0001% or more, more preferably 0.0002% or more, and further preferably 0.0003% or more.

### Mg: 0.0500% or less

As in Ca, Mg (magnesium) forms a compound with S to reduce the amount of S in a matrix, producing an effect of improving hot workability, and therefore, Mg may be contained as necessary. However, an excessive content of Mg leads to a reduction in the amount of S in alloy that contributes to the improvement of the creep rupture strength, which is the advantageous effect of the present invention, and due to being combined with O, leads to a significant degradation of cleanliness, and what is worse, the degradation of hot workability. Accordingly, the content of Mg is 0.0500% or less. The content of Mg is preferably 0.0450% or less. When it is desirable to obtain the above-described effects, the content of Mg is preferably 0.0001% or more, more preferably 0.0002% or more, and further preferably 0.0003% or more.

### REM: 0.1000% or less

As in Ca, REM (rare earth metal) forms a compound with S to reduce the amount of S in a matrix, producing an effect of improving hot workability, and therefore, REM may be contained as necessary. However, an excessive content of REM leads to a reduction in the amount of S in alloy that contributes to the improvement of the creep rupture strength, which is the advantageous effect of the present invention, and due to being combined with O, leads to a significant degradation of cleanliness, and what is worse, the degradation of hot workability. Accordingly, the content of REM is 0.1000% or less. The content of REM is preferably 0.0800% or less. When it is desirable to obtain the above-described effects, the content of REM is preferably 0.0001% or more, more preferably 0.0002% or more, and further preferably 0.0003% or more.

REM is a collective term for a total of 17 elements of Sc, Y, and lanthanoid, and the content of REM refers to a total content of one or more elements of the REM. Furthermore, REM is generally contained in misch metal. Accordingly, for example, the amount of REM may be adjusted into the above-described range by adding the REM in the form of misch metal.

### Co: 1.000% or less

Co (cobalt) has a function of improving the creep rupture strength. That is, as in Ni, Co is an austenite forming element, increases phase stability and contributes to the improvement of the creep rupture strength. Accordingly, Co may be contained. However, Co is a highly expensive element, and therefore, excessively contained Co leads to a significant increase in costs. Accordingly, the content of Co is 1.000% or less. The content of Co is preferably 0.800% or less, and more preferably 0.600% or less. On the other hand, when it is desirable to obtain the above-described effects, the content of Co is preferably 0.010% or more, and more preferably 0.050% or more.

### Cu: 1.00% or less

Cu (copper) has a function of improving the creep rupture strength. That is, as in Ni and Co, Cu is an austenite forming element, increases phase stability and contributes to the improvement of the creep rupture strength. Accordingly, Cu may be contained. However, when Cu is excessively contained, hot workability degrades. Accordingly, the content of Cu is 1.00% or less. The content of Cu is preferably 0.80% or less, and more preferably 0.60% or less. On the other hand, when it is desirable to obtain the above-described effects, the content of Cu is preferably 0.01% or more, and more preferably 0.05% or more.

### Mo: 1.000% or less

Mo (molybdenum) has a function of improving the creep rupture strength. That is, Mo is dissolved in a matrix and has a function of improving the creep rupture strength at high temperature. Accordingly, Mo may be contained. However, when Mo is excessively contained, the stability of austenite degrades, and what is worse, the creep rupture strength degrades. Accordingly, the content of Mo is 1.000% or less. The content of Mo is preferably 0.800% or less, and more preferably 0.700% or less. On the other hand, when it is desirable to obtain the above-described effects, the content of Mo is preferably 0.010% or more, and more preferably 0.050% or more.

### V: 0.500% or less

V (vanadium) has a function of improving the creep rupture strength. That is, as in Nb, V is combined with C, or C and N, forms fine carbide or carbo-nitride, and has a function of improving the creep rupture strength. Accordingly, V may be contained. However, when V is excessively contained, it precipitates in large amounts as carbide or carbo-nitride, and the creep rupture ductility degrades. Accordingly, the content of V is 0.500% or less. The content of V is preferably 0.400% or less, and more preferably 0.300% or less. On the other hand, when it is desirable to obtain the above-described effects, the content of V is preferably 0.010% or more, and more preferably 0.050% or more.

### 2. Formula (i)

As described above, with Cr, W, Fe, and Ni being sufficiently dissolved, it is possible to allow precipitates that contain these elements to finely precipitate in a usage environment, so that an excellent creep rupture strength can be obtained. Accordingly, it is necessary to ensure that, in the alloy member, Cr, W, Fe, and Ni are sufficiently contained in total whereas the amount of Cr, W, Fe, and Ni that are present as precipitates is lowered in advance before being used, and specifically, it is necessary to satisfy the following Formula (i):
$97.50 \leq \left(Cr+W+Fe+Ni\right) - \left({Cr}_{ER}+{W}_{ER}+{Fe}_{ER}+{Ni}_{ER}\right)$
where each symbol in the formulas is defined as below, and each element symbol in the formulas represents a content of each element (mass%) contained in the alloy member,
Cr_{ER}: the content of Cr (mass%) in precipitates obtained by extracted residue analysis
W_{ER}: the content of W (mass%) in precipitates obtained by extracted residue analysis
Fe_{ER}: the content of Fe (mass%) in precipitates obtained by extracted residue analysis
Ni_{ER}: the content of Ni (mass%) in precipitates obtained by extracted residue analysis.

When the right value of Formula (i) is less than 97.50, the amount of solid solution of Cr, W, Fe, and Ni is insufficient, and therefore, the creep rupture strength cannot be improved. Accordingly, the right value of Formula (i) is 97.50 or more. The right value of Formula (i) is preferably 98.00 or more, and more preferably 98.50 or more.

The content of each element (mass%) in precipitates to be analyzed as extraction residues in the above formula can be measured according to the procedure as described below. Specifically, by using 10% acetylacetone - 1% tetramethylammonium chloride / methanol, a sample of about 0.4 g is electrolyzed at a current value of 20 mA/cm². Thereafter, a solution of the electrolyzed sample is filtered through a 0.2 µm filter, followed by acid decomposition of the residues. Then, an ICP (high frequency inductively coupled plasma) optical emission spectrometer is used to calculate a quantity (mass%) analyzed as extraction residues for the above-described elements.

### 3. Formula (ii)

As described above, the inventors have found that there is a certain relationship between the thickness of a member and the grain diameter that leads to a better creep rupture ductility. Specifically, as a result of studies conducted on the relationship between the thickness of a member and the grain diameter that leads to a better creep rupture ductility based on a large amount of experimental data, it has been found that a sufficient creep rupture ductility can be secured by satisfying the following Formula (ii):
$- 2.2 \times {10}^{- 5} \times {t}^{3} + 2.1 \leq D$ where t in the formulas is defined as the thickness of alloy member (mm), and D as the average grain size at a thickness-center portion of the alloy member.

When the average grain size D does not satisfy Formula (ii), austenite grains are coarse, so that the creep rupture ductility cannot be improved. The maximum value of the average grain size D is not particularly limited, whereas when austenite grains are fine, there may be a case in which the above Formula (i) is not satisfied due to an insufficient solution heat treatment, which will be described later. Accordingly, the average grain size D is preferably 6.0 or less, and more preferably 5.0 or less. Furthermore, the average grain size D is preferably -2.0 or more, more preferably -1.0 or more, and further preferably 0 or more.

The average grain size D is measured in compliance with ASTM E112 (2013). Specifically, specimens for microstructural observation are collected such that a section that is perpendicular to the longitudinal direction of the alloy member is an observation surface, and then the observation surface is subjected to mirror polishing. After polishing, etching in mixed acid is carried out, followed by observation with an optical microscope. Observations are made at 10 visual fields such that the thickness-center position of the alloy member is brought into the center of the visual field. Then, the grain size of each visual field is determined according to the comparison method defined in ASTM E112, and the average value of them is determined as average grain size D. At this time, 100× is taken as a reference observation magnification, and 200× or 400× is selected depending on the grain size. When 200× or 400× is selected as the observation magnification, a correction is made in compliance with ASTM E112 (2013) by using a correction value Q defined by the following formula (I): $Q = 6.64 {log}_{10} \left(M/100\right)$ where M in the above formula is an observation magnification.

### 4. Dimension

For example, the austenitic heat resistant alloy member of the present invention may be an alloy tube or an alloy plate. When the austenitic heat resistant alloy member is an alloy tube, the wall thickness is preferably 1 mm or more, or 5 mm or more, and preferably 100 mm or less, 80 mm or less, 65 mm or less, or 55 mm or less. Furthermore, when the austenitic heat resistant alloy member is an alloy plate, the plate thickness is preferably 1 to 100 mm.

### 5. Production Method

While no particular limitation is placed on the production method for the austenitic heat resistant alloy member of the present invention, for example, an ingot or a cast piece that has the above-described chemical composition is subjected to hot working, followed by different types of hot working such as hot extrusion as necessary, and thereafter, a solution heat treatment is carried out. Furthermore, cold working may be carried out as necessary.

As described above, to achieve both excellent creep rupture strength and creep rupture ductility, it is necessary to strictly control the solution heat treatment conditions in consideration of the thickness of the member. Specifically, it is necessary that the solution heat treatment temperature T is 1180 to 1250°C, and the following Formulas (iii) and (iv) are satisfied. After the solution heat treatment, the alloy member is preferably water-cooled.$16.1 \times t + 28500 \leq LMP \leq 16.1 \times t + 29100$ $LMP = \left(T+273.15\right) \times \left(Log \left({t}_{r}\right)+20\right)$ where each symbol in the formulas is defined as below,
t: the thickness of alloy member (mm)
T: solution heat treatment temperature (°C)
tᵣ: solution heat treatment time (h).

When the solution heat treatment temperature T is less than 1180°C, recrystallization does not occur, so that strain caused by working cannot be eliminated, leading to the degradation of the creep rupture ductility. In addition, Cr, W, Fe, and Ni cannot sufficiently be dissolved, and therefore, a better creep rupture strength cannot be secured. On the other hand, when the solution heat treatment temperature T is more than 1250°C, the creep rupture ductility degrades due to coarsening of austenite grains. Accordingly, the solution heat treatment temperature T is 1180 to 1250°C.

When the solution heat treatment time tᵣ is less than 10 min, Cr, W, Fe, and Ni cannot sufficiently be dissolved, and therefore, a better creep rupture strength cannot be secured. Accordingly, the solution heat treatment time tᵣ is 10 min or more.

Furthermore, when LMP (Larson Miller Parameter) defined by Formula (iv) is less than the left value of Formula (iii), Cr, W, Fe, and Ni cannot sufficiently be dissolved, and therefore, a better creep rupture strength cannot be secured. On the other hand, the LMP defined by Formula (iv) is more than the right value of Formula (iii), the creep rupture ductility degrades due to coarsening of austenite grains. Accordingly, it is necessary that the LMP defined by Formula (iv) satisfies Formula (iii).

Hereinunder, the present invention will more specifically be described with reference to examples, whereas the present invention is not limited to the examples.

### EXAMPLE

Austenitic heat resistant alloys 1 to 38, each of which had the chemical composition indicated in Table 1 and Table 2, were melted in a laboratory to fabricate ingots. The ingots were then shaped through hot forging and hot rolling, followed by solution heat treatments under conditions indicated in Table 3 and Table 4, so that alloy tubes (Test Nos. 1 to 50), each of which had a wall thickness as indicated in Table 3 and Table 4, were obtained.

### <Extraction Residues>

The contents (mass%) of Cr, W, Fe, and Ni in precipitates analyzed as extraction residues were measured according to the procedure as described below. Specifically, by using 10% acetylacetone - 1% tetramethylammonium chloride / methanol, a sample of about 0.4 g was electrolyzed at a current value of 20 mA/cm². Thereafter, a solution of the electrolyzed sample was filtered through a 0.2 µm filter, followed by acid decomposition of the residues. Then, an ICP optical emission spectrometer was used to calculate a quantity (mass%) analyzed as extraction residues for the above-described elements.

### <Average Grain Size>

The average grain size D was measured in compliance with ASTM E112 (2013). Specifically, specimens for microstructural observation were collected such that a section that was perpendicular to the longitudinal direction of the alloy tube was an observation surface, and then the observation surface was subjected to mirror polishing. After polishing, etching in mixed acid was carried out, followed by observation with an optical microscope. Observations were made at 10 visual fields in such a way that the wall-thickness-center position of the alloy tube was brought into the center of the visual field. Then, the grain size of each visual field was determined according to the comparison method defined in ASTM E112, and the average value of them was determined as average grain size D. At this time, 100× was taken as a reference observation magnification, and 200× or 400× was selected depending on the grain size. When 200× or 400× was selected as the observation magnification, a correction was made in compliance with ASTM E112 (2013) by using a correction value Q defined by the following formula (I): $Q = 6.64 {log}_{10} \left(M/100\right)$ where M in the above formula is an observation magnification.

### <Creep Rupture Strength and Creep Rupture Ductility>

Next, creep rupture specimens, each of which was a round bar having a diameter of 6 mm and a gage length of 30 mm, were collected from a wall-thickness-center portion of each alloy tube, and creep rupture tests were conducted under conditions of 750°C and 100 MPa. Then, those that exceeded 2000 hours in the creep rupture time were determined to have passed and have a better creep rupture strength. Furthermore, those that exceeded 10% in the reduction of area after creep rupture were determined to have passed and have a better creep rupture ductility.

The results are collectively shown in Table 3 and Table 4. Note that "-" of Test No. 44 in Table 4 means that determination of the grain size was difficult because recrystallization did not occur.

### [Table 3]

**Table 3**

| Test No. | Alloy | Wall thickness t (mm) | Solution heat treatment temperature T(°C) | Solution heat treatment time tr (min) | Left value of Formula (iii) | LMP | Right value of Formula (iii) | Cr+W+ Fe+Ni (mass%) | Cr_{ER}+W_{ER}+ Fe_{ER}+Ni_{ER} (mass%) | Right value of Formula (i) | Left value of Formula (ii) | Average grain size D | Creep rupture time (h) | Creep rupture reduction (%) | |
|---|---|---|---|---|---|---|---|---|---|---|---|---|---|---|---|
| 1 | 1 | 8 | 1210 | 30 | 28629 | 29217 | 29229 | 98.29 | 0.26 | 98.03 | 2.1 | 3.2 | 3277 | 34.5 | |
| 2 | 2 | 8 | 1220 | 10 | 28629 | 28701 | 29229 | 98.24 | 0.16 | 98.08 | 2.1 | 3.5 | 3201 | 29.6 | |
| 3 | 3 | 15 | 1230 | 10 | 28742 | 28893 | 29342 | 98.18 | 0.06 | 98.12 | 2.0 | 4.1 | 3509 | 23.1 | |
| 4 | 4 | 19 | 1210 | 20 | 28806 | 28955 | 29406 | 97.63 | 0.12 | 97.51 | 2.0 | 2.2 | 2135 | 31.4 | |
| 5 | 5 | 11 | 1230 | 15 | 28677 | 29158 | 29277 | 98.02 | 0.27 | 97.75 | 2.1 | 3.3 | 3441 | 25.9 | |
| 6 | 6 | 11 | 1210 | 20 | 28677 | 28955 | 29277 | 98.00 | 0.35 | 97.65 | 2.1 | 3.4 | 2038 | 34.7 | |
| 7 | 7 | 38 | 1240 | 20 | 29112 | 29541 | 29712 | 97.78 | 0.12 | 97.66 | 0.9 | 2.4 | 2451 | 19.3 | |
| 8 | 8 | 48 | 1250 | 10 | 29273 | 29278 | 29873 | 97.72 | 0.09 | 97.63 | -0.3 | 0.5 | 2437 | 15.2 | |
| 9 | 9 | 48 | 1220 | 30 | 29273 | 29414 | 29873 | 97.82 | 0.26 | 97.56 | -0.3 | 0.7 | 2169 | 35.8 | |
| 10 | 10 | 38 | 1220 | 30 | 29112 | 29414 | 29712 | 97.72 | 0.21 | 97.51 | 0.9 | 2.2 | 2471 | 37.3 | |
| 11 | 11 | 38 | 1210 | 30 | 29112 | 29217 | 29712 | 97.64 | 0.13 | 97.51 | 0.9 | 1.9 | 2387 | 30.9 | |
| 12 | 12 | 48 | 1220 | 30 | 29273 | 29414 | 29873 | 97.79 | 0.16 | 97.63 | -0.3 | 0.6 | 2469 | 28.1 | Inventive example |
| 13 | 13 | 48 | 1230 | 30 | 29273 | 29611 | 29873 | 98.10 | 0.06 | 98.04 | -0.3 | 1.1 | 2355 | 22.1 | |
| 14 | 14 | 26 | 1210 | 20 | 28919 | 28955 | 29519 | 97.98 | 0.38 | 97.60 | 1.7 | 3.4 | 2471 | 33.4 | |
| 15 | 15 | 26 | 1180 | 60 | 28919 | 29063 | 29519 | 99.79 | 0.29 | 98.50 | 1.7 | 2.2 | 3822 | 50.7 | |
| 16 | 16 | 8 | 1210 | 20 | 28629 | 28955 | 29229 | 97.84 | 0.20 | 97.64 | 2.1 | 3.0 | 2246 | 37.4 | |
| 17 | 17 | 8 | 1240 | 10 | 28629 | 29086 | 29229 | 98.11 | 0.30 | 97.81 | 2.1 | 3.9 | 2437 | 21.3 | |
| 18 | 18 | 5 | 1240 | 10 | 28581 | 29086 | 29181 | 98.06 | 0.24 | 97.82 | 2.1 | 4.1 | 3098 | 13.7 | |
| 19 | 19 | 5 | 1220 | 10 | 28581 | 28701 | 29181 | 97.79 | 0.23 | 97.56 | 2.1 | 4.0 | 2213 | 34.1 | |
| 20 | 20 | 6 | 1220 | 20 | 28597 | 29151 | 29197 | 98.03 | 0.13 | 97.90 | 2.1 | 3.8 | 2349 | 22.8 | |
| 21 | 21 | 6 | 1230 | 10 | 28597 | 28893 | 29197 | 97.73 | 0.21 | 97.52 | 2.1 | 2.8 | 2471 | 26.4 | |
| 22 | 22 | 19 | 1240 | 10 | 28806 | 29086 | 29406 | 97.65 | 0.13 | 97.52 | 2.0 | 3.3 | 2219 | 22.0 | |
| 23 | 23 | 8 | 1230 | 10 | 28629 | 28893 | 29229 | 97.81 | 0.28 | 97.53 | 2.1 | 4.7 | 2391 | 23.7 | |
| 24 | 24 | 8 | 1230 | 10 | 28629 | 28893 | 29229 | 97.91 | 0.20 | 97.71 | 2.1 | 4.6 | 2861 | 29.1 | |

| | | | | | | | | | | | | | | | |
|---|---|---|---|---|---|---|---|---|---|---|---|---|---|---|---|
| 97.50≦(Cr+W+Fe+Ni)-(Cr_{ER}+W_{ER}+Fe_{ER}+Ni_{ER}) ...(i) -2.2×10⁻⁵×t³+2.1≦D ...(ii) 16.1×t+28500≤LMP≦16.1×t+29100 ...(iii) LMP=(T+273.15)×((Log(tr)+20) ...(iv) | | | | | | | | | | | | | | | |

### [Table 4]

**Table 4**

| Test No. | Alloy | Wall thickness t(mm) | Solution heat treatment temperature T(°C) | Solution heat treatment time tr (min) | Left value of Formula (iii) | LMP | Right value of Formula (iii) | Cr+W+ Fe+Ni (mass%) | Cr_{ER}+W_{ER}+ Fe_{ER}+Ni_{ER} (mass%) | Right value of Formula (i) | Left value of Formula (ii) | Average grain size D | Creep rupture time (h) | Creep rupture reduction (%) | |
|---|---|---|---|---|---|---|---|---|---|---|---|---|---|---|---|
| 25 | 25 | 8 | 1220 | 10 | 28629 | 28701 | 29229 | 97.62 | 0.10 | 97.52 | 2.1 | 4.6 | 2285 | 31.7 | |
| 26 | 26 | 8 | 1220 | 10 | 28629 | 28701 | 29229 | 97.96 | 0.37 | 97.59 | 2.1 | 4.1 | 2793 | 25.5 | |
| 27 | 27 | 35 | 1230 | 30 | 29064 | 29611 | 29664 | 97.76 | 0.21 | 97.55 | 1.2 | 1.9 | 2277 | 19.1 | |
| 28 | 28 | 80 | 1250 | 30 | 29788 | 30004 | 30388 | 98.56 | 0.26 | 98.30 | -9.2 | 1.1 | 2116 | 16.7 | |
| 29 | 29 | 60 | 1250 | 30 | 29466 | 30004 | 30066 | 98.19 | 0.39 | 97.80 | -2.7 | 0.8 | 2357 | 15.5 | |
| 30 | 30 | 8 | 1200 | 30 | 28629 | 29020 | 29229 | 98.13 | 0.31 | 97.82 | 2.1 | 4.7 | 2339 | 37.1 | |
| 31 | 31 | 8 | 1200 | 30 | 28629 | 29020 | 29229 | 97.95 | 0.35 | 97.60 | 2.1 | 4.8 | 2581 | 31.6 | |
| 32 | 32 | 19 | 1210 | 20 | 28806 | 28955 | 29406 | 98.19 | 0.41 | 97.78 | 2.0 | 3.9 | 2506 | 29.8 | |
| 33 | 33 | 19 | 1210 | 20 | 28806 | 28955 | 29406 | 97.96 | 0.18 | 97.78 | 2.0 | 2.8 | 2360 | 33.3 | Inventive example |
| 34 | 34 | 23 | 1230 | 20 | 28870 | 29346 | 29470 | 97.78 | 0.13 | 97.65 | 1.8 | 4.3 | 2497 | 38.1 | |
| 35 | 35 | 35 | 1230 | 20 | 29064 | 29346 | 29664 | 98.13 | 0.22 | 97.91 | 1.2 | 4.1 | 2991 | 34.2 | |
| 36 | 36 | 35 | 1220 | 20 | 29064 | 29151 | 29664 | 98.19 | 0.27 | 97.92 | 1.2 | 3.4 | 2334 | 23.4 | |
| 37 | 37 | 48 | 1220 | 30 | 29273 | 29414 | 29873 | 97.74 | 0.15 | 97.59 | -0.3 | 2.4 | 2401 | 24.5 | |
| 38 | 38 | 48 | 1220 | 30 | 29273 | 29414 | 29873 | 97.73 | 0.16 | 97.57 | -0.3 | 2.6 | 2346 | 21.1 | |
| 39 | 1 | 10 | 1230 | 10 | 28661 | 28893 | 29261 | 98.29 | 0.26 | 98.03 | 2.1 | 4.7 | 2213 | 30.8 | |
| 40 | 2 | 20 | 1240 | 10 | 28822 | 29086 | 29422 | 98.24 | 0.23 | 98.01 | 1.9 | 4.6 | 2267 | 28.0 | |
| 41 | 3 | 30 | 1240 | 20 | 28983 | 29541 | 29583 | 98.18 | 0.16 | 98.02 | 1.5 | 4.4 | 3071 | 40.8 | |
| 42 | 4 | 40 | 1240 | 20 | 29144 | 29541 | 29744 | 97.63 | 0.09 | 97.54 | 0.7 | 1.8 | 3220 | 16.8 | |
| 43 | 5 | 50 | 1250 | 20 | 29305 | 29736 | 29905 | 98.02 | 0.11 | 97.91 | -0.7 | 0.8 | 3001 | 13.7 | |
| 44 | 1 | 8 | 1160 | 10 | 28629 | 27548 | 29229 | 98.29 | 1.07 | 97.22 | 2.1 | - | 1873 | 7.9 | |
| 45 | 4 | 19 | 1210 | 10 | 28806 | 28509 | 29406 | 97.63 | 0.54 | 97.09 | 2.0 | 4.5 | 1921 | 20.1 | |
| 46 | 6 | 11 | 1240 | 30 | 28677 | 29807 | 29277 | 98.00 | 0.11 | 97.89 | 2.1 | -0.5 | 2551 | 6.6 | Comparative example |
| 47 | 7 | 38 | 1270 | 20 | 29112 | 30127 | 29712 | 97.78 | 0.26 | 97.52 | 0.9 | -2.0 | 3811 | 4.1 | |
| 48 | 10 | 35 | 1200 | 10 | 29064 | 28317 | 29664 | 97.72 | 0.49 | 97.23 | 1.2 | 6.7 | 1628 | 24.1 | |
| 49 | 8 | 48 | 1100 | 30 | 29273 | 27050 | 29873 | 97.72 | 1.25 | 96.47 | -0.3 | 7.2 | 1540 | 8.7 | |
| 50 | 3 | 15 | 1200 | 5 | 28742 | 27873 | 29342 | 98.18 | 1.44 | 96.74 | 2.0 | 5.7 | 1891 | 22.7 | |

| | | | | | | | | | | | | | | | |
|---|---|---|---|---|---|---|---|---|---|---|---|---|---|---|---|
| 97.50≦(Cr+W+Fe+Ni)-(Cr_{ER}+W_{ER}+Fe_{ER}+Ni_{ER}) ...(i) 16.1×t+28500≦LMP≦16.1×t+29100 ...(iii) -2.2×10⁻⁵×t³+2.1≦D ...(ii) LMP=(T+273.15)×((Log(tr)+20) ...(iv) The underline indicates that the value fell out of the requirements of the present invention. | | | | | | | | | | | | | | | |

As shown in Table 3 and Table 4, Test Nos. 1 to 43, which satisfied all the provisions of the present invention, produced better results for both the creep rupture strength and the creep rupture ductility. In contrast, in Test No. 44, the creep rupture ductility degraded because the solution heat treatment temperature T was low, and therefore, recrystallization did not occur. In addition, LMP was less than the left value of Formula (iii), and therefore, Cr, W, Fe, and Ni could not sufficiently be dissolved, leading to the degradation of the creep rupture strength.

In Test Nos. 45 and 48, LMP was less than the left value of Formula (iii), and therefore, Cr, W, Fe, and Ni could not sufficiently be dissolved, leading to the degradation of the creep rupture strength. In Test No. 46, LMP was more than the right value of Formula (iii), and therefore, the average grain size D was lower than the left value of Formula (ii), leading to the degradation of the creep rupture ductility. In Test No. 47, the solution heat treatment temperature T was high and LMP was more than the right value of Formula (iii), and therefore, the average grain size D was lower than the left value of Formula (ii), leading to the degradation of the creep rupture ductility. In Test No. 49, the solution heat treatment temperature T was low, and therefore, recrystallization did not occur, leading to the degradation of the creep rupture ductility. In addition, Cr, W, Fe, and Ni could not sufficiently be dissolved, leading to the degradation of the creep rupture strength. In Test No. 50, the solution heat treatment time tᵣ was short, and therefore, Cr, W, Fe, and Ni could not sufficiently be dissolved, leading to the degradation of the creep rupture strength.

### INDUSTRIAL APPLICABILITY

The austenitic heat resistant alloy member of the present invention is excellent in both the creep rupture strength and the creep rupture ductility for a long time. Accordingly, the austenitic heat resistant alloy member of the present invention is suitably used as a material for superheater tubes or reheater tubes of power generation boilers.

## Claims

1. An austenitic heat resistant alloy member having a chemical composition comprising, in mass%:
C: 0.010 to 0.150%,
Si: 2.00% or less,
Mn: 2.00% or less,
P: 0.0400% or less,
S: 0.0100% or less,
Cr: 20.00 to 28.00%,
Ni: 35.00 to 50.00%,
W: 4.00 to 10.00%,
Ti: 0.01 to 1.20%,
Nb: 0.01 to 1.00%,
N: 0.0200% or less,
Al: 0.010 to 0.300%,
B: 0.0005 to 0.0400%,
O: 0.0100% or less, and
the balance: Fe and impurities, and
satisfies following Formulas (i) and (ii): $97.50 \leq \left(Cr+W+Fe+Ni\right) - \left({Cr}_{ER}+{W}_{ER}+{Fe}_{ER}+{Ni}_{ER}\right)$ $- 2.2 \times {10}^{- 5} \times {t}^{3} + 2.1 \leq D$
where each symbol in the formulas is defined as below, and each element symbol in the formulas represents a content of each element (mass%) contained in the alloy member,
Cr_{ER}: a content of Cr (mass%) in precipitates obtained by extracted residue analysis
W_{ER}: a content of W (mass%) in precipitates obtained by extracted residue analysis
Fe_{ER}: a content of Fe (mass%) in precipitates obtained by extracted residue analysis
Ni_{ER}: a content of Ni (mass%) in precipitates obtained by extracted residue analysis
t: a thickness of the alloy member (mm)
D: an average grain size at a thickness-center portion of the alloy member.

2. The austenitic heat resistant alloy member according to claim 1, wherein in lieu of a part of the Fe, the chemical composition contains one or more elements, in mass%, selected from:
Ca: 0.0100% or less,
Mg: 0.0500% or less,
REM: 0.1000% or less,
Co: 1.000% or less,
Cu: 1.00% or less,
Mo: 1.000% or less, and
V: 0.500% or less.
